

## UNITED STATES PATENT OFFICE

2,506,301

## RECOVERY OF RESINS FROM COAL

Ernest Klepetko and Philip de B. Kaye, Bauer,  
and Lester J. Hartzell, Jr., Tooele, Utah, assign-  
ors to Combined Metals Reduction Company,  
Stockton, Utah, a corporation of Utah

No Drawing. Application June 17, 1946,  
Serial No. 677,394

8 Claims. (Cl. 260—107)

1

This invention relates to the recovery of resins from coal, and is particularly directed to the production of a resin concentrate by flotation from resin-bearing coal. The invention has for its principal objects to produce a resin flotation concentrate which is easily amenable to further refining (as by solvent extraction), and to produce a salable coal residue. These objects are achieved in accordance with the complete process of the invention by controlled crushing of the coal preparatory to flotation, by proper control of the pulp density of the coal-bearing pulp during flotation, and by conducting the flotation operation in the absence of mechanical agitation of the pulp.

Some coal deposits contain a substantial quantity of a natural fossil resin which, in purified condition, is suitable for use in varnishes, in printing inks, in the manufacture of resinous waterproofing agents, in synthetic rubber compositions and rubber cements, and in similar resin-containing products. The resin, however, is quite intimately admixed with the coal, and the problem of separating it from the coal economically and on a commercial scale has presented serious difficulties. In United States Patent No. 1,773,997, granted August 26, 1930, to William D. Green, it is pointed out that solvent extraction of the resin directly from the coal is wasteful of the solvent, and that separation by means of a liquid of high specific gravity is accompanied by substantial mechanical loss of the liquid used and contamination of the products. Sink-and-float processes more recently proposed are not effective for adequate and efficient recovery of the finer resin particles. Green proposed separating the resin by a flotation process, using one of the high alcohols, turpentine, cresol, one of the pine oils, or the like, as the flotation agent.

Green's process is effective for producing a flotation concentrate containing a high percentage of resin, but the resin concentrate is not sufficiently pure for most commercial uses without further refining. Refining by solvent extraction is particularly desirable, because the resin is unaffected by the solvent extraction treatment, and when a resin flotation concentrate is used as the raw material in a cyclic solvent extraction process, the consumption of solvent is economically low. Practically, however, solvent extraction refining of a resin flotation concentrate produced in accordance with Green's method is very difficult, because the insoluble coal contaminants in the resin concentrate are so fine that they cannot be separated economically and efficiently from a solution of the resin in a solvent. Although this insoluble matter constitutes only a small percentage by weight of the concentrate, it is present in such a fine state of comminution

2

that it will not settle on standing, and quickly plugs up the pores of any satisfactory commercial filter medium.

In the course of an exhaustive investigation of this problem, we have determined that the resin is far more friable than the coal with which it is admixed. In addition, careful examination of numerous coal samples from a number of mines has disclosed that the resin occurs in fracture planes of various thicknesses, and that the finest resin grains in these planes ordinarily are of about 40-mesh size. Our investigations have revealed that, owing to the friability of the resin and the consequent tendency of the coal to fracture along the resin seams, and to the fact that the resin particles in the coal are not excessively fine, substantially all of the resin is liberated from its mechanical bond to the coal if the coal is crushed only enough to pass a 6-mesh to 8-mesh screen. We have further discovered that the excessively fine character of the coal impurity present in resin concentrates as heretofore prepared by the Green flotation process is due to unnecessarily fine crushing of the coal preparatory to flotation, and to comminution that occurs by attrition during the course of the flotation operation.

Based on these discoveries, our present invention contemplates crushing the resin-bearing coal no finer than necessary to pass a 6- to 8-mesh screen, and forming a pulp of the crushed product in water. The density of the pulp is adjusted to not more than about 15% by weight of solids, and the resulting pulp is subjected to a flotation operation in an air-agitated flotation unit in the absence of mechanical agitation. The coarse crushing of the coal is adequate to liberate the resin sufficiently for effective flotation, but produces a minimum of fines. Maintaining the pulp density at a low value, below about 15% solids, facilitates settling of such coal fines as are produced and so tends to keep them out of the floated resin concentrate, and in addition, minimizes formation of fines by attrition of the coal particles against one another. Conducting the flotation operation in the absence of mechanical agitation further aids in minimizing formation of fines by attrition of the particles in the pulp. (The term "mechanical agitation" is used herein to denote agitation by a mechanical stirring device, such as an impeller, as distinguished from the agitation that occurs from bubbling air through the pulp, or in the course of its flow through the equipment of the flotation plant). Thus the foregoing features each contribute to avoiding formation of coal fines and to preventing accumulation of this objectionable impurity in the resin concentrate. When used in combination, these features permit of producing a resin concentrate having a screen analysis approximating at least about 50% plus 100-mesh, and in which the contami-

nating particles of coal are therefore sufficiently coarse to be readily amenable to removal during refining of the concentrate by solvent extraction, which involves dissolving the resin from the concentrate in a solvent for the resin and then separating the insoluble coal residue from the solution by filtration, thickening, or otherwise.

The fact that relatively coarse crushing is adequate to liberate the resin sufficiently for substantially complete recovery by flotation was demonstrated by tests conducted on three large batches of coal all obtained from the same source. One batch was reduced by carefully controlled crushing to pass through a 20-mesh screen, a second batch was carefully crushed to pass a 10-mesh screen, and the third batch was reduced by equally careful crushing to pass only a 6-mesh screen. Each batch was separately subjected to a flotation operation using pine oil as the flotation agent. Practically identical resin recoveries were obtained in the flotation concentrate from each batch. Hence it is evident that crushing to the finer sizes is not necessary to secure improved resin recoveries in the flotation concentrate. The physical quality of the concentrates produced from the more coarsely crushed batches of coal was decidedly superior to that of the concentrate obtained from the batch crushed to minus 20-mesh. Moreover, the coal tailing from the more coarsely crushed batches contained a substantially lower percentage of fines than did the tailing from the 20-mesh material, and consequently was a much more readily salable coal product.

These tests establish that crushing no finer than necessary to pass a 6- or 8-mesh screen is ample for obtaining a high resin recovery in the flotation concentrate, and leads to the production of a resin concentrate and a coal tailing having physical properties superior to what can be obtained when the raw material is crushed to the finer sizes heretofore customary in such flotation operations.

The pronounced effect of attrition in producing fines in the course of the flotation operation is demonstrated by the data set forth in Table I. These data were obtained from screen analyses of the solids contained in the feed to a resin flotation operation, and in the tailing and concentrate products. The resin-bearing coal feed was prepared for this operation by controlled graded crushing of a large lot to a 8-mesh size, and the flotation operation was carried out in a standard commercial-size mechanically agitated flotation machine. The screen analyses set forth in the last three columns are expressed in percent solids of the screen size indicated in the first column.

TABLE I

*Screen analysis of flotation machine feed and products*

| Mesh  | Percent Cumulative |         |             |
|-------|--------------------|---------|-------------|
|       | Feed               | Tailing | Concentrate |
| +8    | 1.1                | 0.1     | —           |
| +10   | 17.9               | 1.1     | —           |
| +20   | 41.5               | 5.6     | —           |
| +48   | 71.7               | 10.7    | 0.3         |
| +65   | 77.7               | 16.9    | 1.9         |
| +100  | 83.1               | 37.9    | 6.3         |
| -100  | 16.9               | 62.1    | 93.7        |
| Total | 100.0              | 100.0   | 100.0       |

The excessive attrition which occurred during

the flotation operation is well shown by the foregoing screen analyses. For example, it will be noted that whereas the original feed contained only 16.9% minus 100-mesh, the coal tailing contained almost four times as much (62.1%) minus 100-mesh material, and that the concentrate was almost all (93.7%) minus 100-mesh.

The screen analyses reported in Table I are based on a flotation operation conducted in a mechanically agitated flotation unit. We have found that the attrition and production of fines that occurs during the flotation operation may be greatly reduced if the flotation is conducted in an air-agitated unit. Such air-agitated flotation units are exemplified by the Callow canvas bottom cell, the McIntosh cell with canvas cover air rotor, and the air-lift Forrester type of cell. In general, using the coarsely crushed feed that we prefer to employ, the air-lift type of flotation machine is generally most satisfactory.

In order to compare the attrition characteristics of mechanically agitated flotation units with those of air-agitated flotation units, a batch of coal carefully crushed to pass a 20-mesh screen was subjected to a flotation operation in an air-lift type of cell, and another batch of coal carefully crushed to pass an 8-mesh screen was subjected to a flotation operation in a mechanically agitated cell. The screen analyses obtained for the feed and concentrate in each of these operations is set forth in Table II. Again the screen analyses are expressed in percent solids of the screen size shown in the first column.

TABLE II

*Attrition characteristics of mechanically agitated and air-lift flotation units*

| Mesh  | Feed                              |                                    | Concentrate                       |                                    |
|-------|-----------------------------------|------------------------------------|-----------------------------------|------------------------------------|
|       | Mechan.<br>Per Cent<br>Cumulative | Air-Lift<br>Per Cent<br>Cumulative | Mechan.<br>Per Cent<br>Cumulative | Air-Lift<br>Per Cent<br>Cumulative |
| +28   | 41.5                              | 14.7                               | —                                 | 3.8                                |
| +48   | 71.7                              | 58.0                               | 0.3                               | 21.7                               |
| +65   | 77.5                              | 70.5                               | 1.9                               | 32.5                               |
| +100  | 83.1                              | 79.3                               | 6.3                               | 45.6                               |
| -100  | 16.9                              | 20.7                               | 93.7                              | 54.4                               |
| Total | 100.0                             | 100.0                              | 100.0                             | 100.0                              |

The screen analyses reported in Table II show how much greater is the amount of attrition that occurs in the mechanically agitated cell than in the air-agitated type of cell. In spite of the fact that the air-lift cell was operated on a very much finer feed than the mechanically agitated cell, thus favoring the latter, the concentrate obtained from the air-lift machine contained only 54.4% minus 100-mesh, whereas the concentrate from the mechanically agitated cell contained 93.7% minus 100-mesh. The much coarser concentrate obtained using the air-lift cell in the absence of mechanical agitation (the screen analysis of which concentrate approximated 50% plus 100-mesh) was considerably more amenable to refinement by solvent extraction than was the relatively finer concentrate obtained from the mechanically agitated unit. In addition, the coal tailing produced in the air-lift cell was coarser and more readily salable than was the coal tailing produced in the mechanically agitated cell.

As a matter of interest, the screen analyses set forth in Table II are indicative of how readily friable is the resin contained in the coal. Even

in the case of the air-lift type of machine, with its gentle agitation of the pulp, the screen analysis shows that whereas only 20.7% of the feed (mostly coal) was minus 100-mesh, over 2½ times this amount of the concentrate (mostly resin) was minus 100-mesh. Table I also indicates the friable nature of the resin, in that it shows the much coarser quality of the coal tailing as compared with the resin concentrate from the same flotation unit.

A further important factor which affects the quality of the resin concentrate is the density of the pulp in the flotation circuits. This pulp consists of a water suspension of the solid coal and resin particles, in which the solid particles are in a constant state of random motion induced by agitation and by flow of the pulp. The random motion of the solid particles in the pulp results in frequent collisions between the particles, with consequent attrition and production of fines. The frequency with which collisions occur, and hence the amount of fines produced in this fashion, is to some extent a function of the pulp density. A low pulp density favors avoiding the production of fines. While it is not possible to set a hard and fast maximum limit of pulp density, we have found that, in general, the most satisfactory concentrate for subsequent refining by solvent extraction is obtained if the maximum pulp density employed in the flotation circuit does not exceed about 15% by weight of solids.

The flotation operation may be conducted in two or more steps, employing rougher and cleaner flotation operations. In the rougher operation a coal tailing low in resin content, and a resin middling, are produced. In the cleaner operation, the resin middling from the rougher operation is floated under conditions designed to produce a resin concentrate containing a minimum amount of coal impurities, and a tailing consisting of a mixture of coal and resin which may be returned to the rougher operation for retreatment. The cleaner operation may in turn be conducted in two or more separate cleaner flotation steps to secure production of a high grade resin concentrate.

When conducting the flotation operation in two or more steps as outlined above, it is generally most advantageous to maintain the pulp density in the rougher circuit at a value not above about 15% solids and to conduct the cleaner operations at considerably lower pulp densities. For example, in a three-step flotation operation, employing two cleaner stages, the pulp density in the first cleaner stage advantageously does not exceed about 10% by weight of solids, and it is best if the pulp density in the final cleaner stage does not exceed about 8% by weight of solids.

While a low pulp density promotes production of a clean concentrate free from an objectionably high quantity of fines, commercially efficient conduct of the flotation operation sets practical minimum limits to the pulp densities. If the pulp densities are too low, excessively large volumes of pulp have to be handled, and a large plant is required in relation to the amount of resin concentrate produced. By way of example, advantageous and practical pulp density limits in the several stages of a three-step flotation operation of the character outlined above are about 10% to about 15% by weight of solids in the rougher stage, not over about 10% and not less than about 5% by weight of solids in the first cleaner stage, and not over about 8% and not

less than about 3% by weight of solids in the final cleaner stage.

The total amount of fines appearing in the concentrate (and in the coal tailing) produced in a given flotation unit depends, of course, on the amount of coal slime made in preparing the feed to the first flotation unit, as well as on the pulp densities prevailing during flotation. To some extent, therefore, the optimum pulp density to be employed will be governed, in part at least by the amount of fines initially present in the flotation feed.

Control of the factors that influence fine production is important not only for the purposes of producing a coarse coal tailing and a resin concentrate in which the coal impurities are sufficiently coarse to be readily separated in a refining process, but also to minimize the extent to which coal impurities accumulate in the resin concentrate—that is, to produce a clean concentrate. Due to the low specific gravity of the coal in the pulp, there is always a tendency for very fine coal particles to float over with the resin concentrate. The greater the amount of coal fines present in the flotation pulp, the greater will be the proportion of coal impurities that find their way into the resin concentrate, assuming other conditions remain constant. Proper control of the pulp density is a particularly important factor in this connection, as such control not only aids in minimizing the production of fines by attrition, but is of material consequence in minimizing the tendency of such coal fines as are formed to float with the resin concentrate. For this purpose, the pulp density should at all times be sufficiently low so that substantially free and unhindered settling of the coal particles can occur. It is chiefly for this reason that the pulp density in the cleaner circuits of a multi-stage flotation operation should be considerably lower than in the rougher circuit. The resin middling product which constitutes the feed to the cleaner operations is composed of a much higher proportion of fine material than is the feed to the rougher operation, and the fine coal particles in this product settle less readily than do the coarse coal particles in the rougher pulp. Accordingly a more dilute pulp is necessary in the cleaner stages than in the rougher stage in order to favor settling of the coal fines and so reduce their tendency to float over with the cleaner resin concentrate. With a pulp of properly low density, separation of the coal fines and resin is also favored by the difference in specific gravity between the coal and resin (the specific gravity of the coal ordinarily is about 1.6 and of the resin about 1.2). We have found that pulp densities within the limits set forth above are generally satisfactory for producing a resin concentrate of good commercial quality and low in undesirable coal impurities.

In contrast to accepted procedures for floating sulphide minerals, and in contrast to flotation practice as sometimes employed in coal preparation, it has been found that the resin can be floated to the surface of the pulp without the use of air. However, air introduced into the pulp is a desirable accelerant for bringing the resin to the surface, and accordingly, it is advantageous to conduct the flotation operation in an air-agitated unit in order to secure rapid collection of the resin concentrate. The air admitted to the pulp, especially in a cleaner operation, should not enter so rapidly as to cause a degree of agitation too great to permit fairly ready settling of the coal

fines; for otherwise, as indicated above, it will be difficult to produce a clean resin concentrate.

We have found that a very good grade of resin concentrate, and a readily salable coal tailing, may be produced in the course of a flotation operation conducted as herein described. The coal tailing is coarser, and so generally more acceptable to the trade, than has been produced by heretofore known flotation methods for recovering resins from coal. A good recovery of resin in the concentrate is attained, and the concentrate is high in resin content and of excellent physical characteristics for subsequent refining by solvent extraction or otherwise. While it is not generally economic to degrade coarse coal, such as nut or lump coal, by crushing merely to liberate and recover its resin content, the flotation method herein described may be applied economically to the finer coal screenings. In addition to recovering the resin as a valuable by-product, the coal tailing is itself beneficiated by removal of the resin, because the resin yields a lesser number of heat units per pound when burned than does the coal itself.

We claim:

1. In a process for the recovery of a resin from resin-bearing coal involving crushing the coal, subjecting the crushed coal to a flotation operation to prepare a resin concentrate, leaching the concentrate with a solvent for the resin, and separating the resulting resin solution from the insoluble constituents of the concentrate, the improvement which comprises crushing the resin-bearing coal no finer than necessary to pass a 6- to 8-mesh screen and forming a pulp of the crushed product in water, adjusting the density of the pulp to no more than about 15% by weight of solids, and subjecting the resulting pulp to the flotation operation in an air-agitated flotation unit and in the absence of mechanical agitation of the pulp, whereby when the resin concentrate is leached the resin solution thereby obtained is readily separated by filtration from the insoluble constituents of the concentrate.

2. In a process for the recovery of a resin from resin-bearing coal involving crushing the coal, subjecting the crushed coal to a flotation operation to prepare a resin concentrate, leaching the concentrate with a solvent for the resin, and separating the resulting resin solution from the insoluble constituents of the concentrate, the improvement which comprises crushing the resin-bearing coal no finer than necessary to pass a 6- to 8-mesh screen and forming a pulp of the crushed product in water, adjusting the density of the pulp to no more than about 15% by weight of solids, subjecting the resulting pulp to a rougher flotation operation in an air-agitated flotation unit and in the absence of mechanical agitation of the pulp, separating and recovering the rougher coal tailing, separating the rougher resin concentrate product and incorporating it in a pulp having a density no greater than about 10% by weight of solids, and subjecting the resulting pulp to a cleaner flotation operation in a second air-agitated flotation unit and in the absence of mechanical agitation, whereby when the resin concentrate is leached the resin solution thereby obtained is readily separated by filtration from the insoluble constituents of the concentrate.

3. In a process for the recovery of a resin from resin-bearing coal involving crushing the coal, subjecting the crushed coal to a flotation operation to prepare a resin concentrate, leaching the

concentrate with a solvent for the resin, and separating the resulting resin solution from the insoluble constituents of the concentrate, the improvement which comprises forming a pulp of the crushed coal in water, adjusting the density of the pulp to a value no greater than about 15% by weight of solids, and subjecting the pulp at such density to a flotation operation to produce a resin concentrate and a coal tailing, whereby when the resin concentrate is leached the resin solution thereby obtained is readily separated by filtration from the insoluble constituents of the concentrate.

4. In a process for the recovery of a resin from a resin-bearing coal, involving subjecting a pulp containing the resin-bearing coal to rougher and cleaner flotation operations to prepare a resin concentrate and leaching said concentrate with a solvent for the resin, the improvement which comprises maintaining the pulp density in the rougher flotation operation at a value no higher than about 15% by weight of solids, and maintaining the pulp density in the cleaner flotation operation at a value no higher than about 10% by weight of solids, whereby when the resin concentrate is leached the resin solution thereby obtained is readily separated by filtration from the insoluble constituents of the concentrate.

5. In a process for the recovery of a resin from a resin-bearing coal involving crushing the coal, subjecting the crushed coal to a flotation operation to prepare a resin concentrate, leaching the concentrate with a solvent for the resin, and separating the resulting resin solution from the insoluble constituents of the concentrate, the improvement which comprises conducting the flotation in an air-agitated flotation unit in the absence of mechanical agitation, whereby when the resin concentrate is leached the resin solution thereby obtained is readily separated by filtration from the insoluble constituents of the concentrate.

6. In a process for the recovery of a resin from a resin-bearing coal, involving crushing the coal, subjecting the crushed coal to a flotation operation to prepare a resin concentrate, leaching the concentrate with a solvent for the resin, and separating the resulting resin solution from the insoluble constituents of the concentrate, the improvement which comprises subjecting the coal in a pulp containing not more than about 15% by weight of solids to a flotation operation in an air-agitated flotation unit in the absence of mechanical agitation, whereby when the resin concentrate is leached the resin solution thereby obtained is readily separated by filtration from the insoluble constituents of the concentrate.

7. In a process for the recovery of a resin from a resin-bearing coal, involving crushing the coal, subjecting the crushed coal to a flotation operation to prepare a resin concentrate, leaching the concentrate with a solvent for the resin, and separating the resulting resin solution from the insoluble constituents of the concentrate, the improvement which comprises crushing the coal no more than necessary to enable the crushed product to pass a 6-mesh screen prior to subjecting it to the flotation operation to produce the resin concentrate, whereby when the concentrate is leached the resin solution thereby obtained is readily separated by filtration from the insoluble constituents of the concentrate.

8. The improvement according to claim 5, characterized in that the pulp density during the

flotation operation is no greater than about 10%  
by weight of solids.

ERNEST KLEPETKO.  
PHILIP DE B. KAYE.  
LESTER J. HARTZELL, JR.

## REFERENCES CITED

The following references are of record in the  
file of this patent:

## UNITED STATES PATENTS

| Number    | Name       | Date          |
|-----------|------------|---------------|
| 1,773,997 | Green      | Aug. 26, 1930 |
| 2,364,090 | Nagelvoort | Dec. 5, 1944  |

## OTHER REFERENCES

- Gaudin, "Flotation," 1932, McGraw Hill Co.,  
117, 118, 120, 121, 122, 131, 139, 140, 142,  
143, 151, 152, 153, 154, 350 to 353.  
American Institute of Mining and Metallurgical  
Engineer, Contribution No. 86, copyright 1935,  
pages 3, 4, 5, 6.  
Denver Equipment Index, 1936, Denver Equipment  
Co., Denver, Colo., pages 104, 105.  
Bureau of Mines Report of Investigations, No.  
3599, 1941, pp. 16.  
Nagelvoort, Chemical and Metallurgical En-  
gineering, Oct. 1942, pp. 80-82.